

## UNITED STATES PATENT OFFICE

2,021,152

## NOVELTY FINISH

Theodore A. Neuhaus, Lakewood, Ohio, assignor  
to The Glidden Company, Cleveland, Ohio, a  
corporation of Ohio

No Drawing. Application February 14, 1934,  
Serial No. 711,273

12 Claims. (Cl. 91—68)

This invention relates to novelty finishes, and has particular reference to a new and novel two-tone metallic finish obtained by the use of a dyed metallic lacquer over a composite undercoater.

5 Two tone finishes have been obtained in the past by various expedients. In all cases, the surface to be finished is first coated with a solid coating of one color, and a second color is then applied so as to cover only part of the undercoater. This 10 may be accomplished by using various types of top coats. The brush, of course, is always available, to form decorative designs. The undercoater may be masked off in the desired design, and an ordinary top coat then sprayed; the masking operation, however, is slow and expensive. 15 Colors may also be fogged on, to give the so-called "antiqued" effect. "Veiling" lacquers may be used, which string out of a spray gun, and stay put in strings on the surface. These give a pleasing 20 design, of a definite type.

A very popular finish some years ago was the so-called "crackle" lacquer. These are highly pigmented lacquers with such low percentages of binder that on application to a surface, the film 25 cracks open. Because of the poor film strength, an undercoater is necessary to give adhesion and strength to the film; and it is almost essential that a top coat be applied to the film, to protect and liven up the dull, porous crackled film. By using 30 contrasting colors for undercoat and crackle lacquer, with a clear top coat, a pleasing two-tone effect can be obtained; using a colored top-coat of well-selected color, a grain effect resembling leather results.

35 It is, however, impossible to obtain a two toned metallic effect by this method. While a metallic undercoater can be used, good crackle lacquers cannot be obtained using metallic powders as pigments. It is possible to get a broken film, but 40 the design is not uniformly crackled. In addition, a clear top coat to protect the lacquer results in a non-metallic effect being obtained.

I have found that a two-tone metallic effect can 45 be obtained by the use of a dyed metallic lacquer as a top coat over crackled lacquer, or over any composite undercoater where a portion of the undercoater is relatively porous, and the other portion is relatively non-porous. The porous portions of the undercoater absorb the dye, separating it from the metal powder, so that over the porous portions the lacquer dries to the color of the metallic powder; over the non-porous portions of the undercoater it dries to a metallic color which depends on the dye used. As no top 50

coat is needed over the bronzing lacquer, a metallic two-tone effect is obtained.

As an example of my invention, I employ as a base coat an ordinary black lacquer, formulating it for the surface to be finished. Regular wood 5 or metal lacquer enamels may be employed. I then spray a black crackle lacquer over the base coat, permitting it to crackle and form a composite undercoater, the base coat showing through the crackle to give a non-porous surface, the 10 crackle lacquer presenting a porous surface. This black crackle may be formulated as follows:

|                                                                                              |    |
|----------------------------------------------------------------------------------------------|----|
| 5 gallons 25% solution of $\frac{1}{2}$ second nitrocellulose<br>in toluol and ethyl acetate | 15 |
| 10 gallons 10% solution of 30-40' second nitro-<br>cellulose in toluol and ethyl acetate     |    |
| 2 gallons 6# dewaxed damar cut in toluol-alcohol                                             |    |
| 8½ gallons toluol                                                                            |    |
| 2½ gallons ethyl acetate                                                                     | 20 |
| 6 gallons anhydrous alcohol                                                                  |    |
| 1½ gallons amyl acetate                                                                      |    |
| 40 carbon black                                                                              |    |
| All ground in a pebble mill overnight to a poor<br>"C" grind.                                | 25 |

I prefer to use the black undercoaters because of low cost; it is possible to use any color on either coat, the only essential being that the base coat dry to a relatively non-porous surface.

Over the composite undercoat I spray my dyed 30 metallic lacquer. The clear lacquer used may be of any composition, and is preferably an ordinary bronzing lacquer using high viscosity nitrocellulose with some gum. A satisfactory lacquer of this type, designed to reduce 100% for spraying 35 may be made from—

|                                                                                           |    |
|-------------------------------------------------------------------------------------------|----|
| 10 ounces of a 17.5% solution of 70% dope nitro-<br>cellulose in toluol and ethyl acetate |    |
| 2 ounces of a 70% solution of ester gum in toluol                                         | 40 |
| 2½ ounces of butanol                                                                      |    |
| 1 ounce of ethyl acetate                                                                  |    |
| 8½ ounces of toluol                                                                       |    |
| 3½ ounces of butyl acetate                                                                |    |

The metal powder used may be of any type, de- 45 pending on the color combination desired. Enough powder should be used for covering (from  $\frac{1}{4}$ #-2# per gallon). If a powder other than aluminum is used, it should be added to the lacquer on the job, as all metallic powders other 50 than aluminum tend to gel the lacquer or change color in the package.

The clear lacquer may be dyed before or after the powder is added. As this addition requires a trained eye and careful shading, I prefer to add 55

it at the factory, so that where powder is to be added on the job, it is added to a ready dyed lacquer. The dyes may be any colors compatible with nitrocellulose lacquers, and should preferably be added in solution. Satisfactory dye solutions are solutions of water soluble acid type dyes in the mono ethyl ether of ethylene glycol and methanol; some oil soluble dyes give satisfactory results with lacquer, and may be used.

10 An indicated above, the dyed metallic lacquer, on being sprayed over the composite undercoater, dries to the dyed metallic color over the non-porous portions of the undercoater, and to the original color of the metal over the porous portions, owing to the absorption of the dye by the porous undercoater. Thus a pleasing two-tone metallic effect is obtained in a simple, economical manner.

While I have applied this invention particularly to crackle lacquer, as a cheap and convenient way of getting a two-tone metallic finish, other methods of obtaining a composite undercoater may be used, such as brushing, or mask spraying, a porous product (such as an iron filler, or a coarsely ground surfacer for example) over a non-porous product.

By using a porous undercoater (such as iron filler or a surfacer) and partially sealing it with a clear sealer, or a non-porous oil, synthetic or lacquer enamel, using a brush, a mask spray or a squeegee application through a silk screen in a manner well known to the art, I obtain a surface in which the design is non-porous, the background porous, thus reversing the metallic contrast when a dyed metallic lacquer is applied.

It is apparent that this invention resides in my discovery that porous surfaces have a selective action on the dye in dyed metallic lacquers, and the application of that discovery to the production of my new finish.

I claim—

1. An article coated with a two-tone metallic finish comprising a composite base coat presenting both porous and non-porous areas, and a top coat containing a metallic powder and dye.
2. An article coated with a two-tone metallic finish comprising a composite base coat presenting both porous and non-porous areas, and a nitrocellulose lacquer top-coat containing a metallic powder and dye.
3. An article coated with a two-tone metallic finish comprising a relatively porous first coat, a non-porous second coat partially sealing the first coat, and a top-coat containing a metallic powder and dye.
4. An article coated with a two-tone metallic finish comprising a relatively non-porous first coat, a porous second coat partially covering the

first coat, and a top-coat containing a metallic powder and dye.

5. An article coated with a two-tone metallic finish comprising a relatively non-porous first coat, a crackled porous second coat, and a top-coat containing a metallic powder and dye.

6. An article coated with a two-tone metallic finish comprising a relatively non-porous first coat, a second coat of crackle lacquer, and a top-coat containing a metallic powder and dye.

7. The method of producing a two-tone metallic finish which comprises preparing a surface presenting both porous and non-porous areas, and applying a top-coat thereon containing a metallic powder and a dye, whereby the top-coat dries to the dyed metallic color over the non-porous areas, and to the undyed metallic color over the porous areas.

8. The method of producing a two-tone metallic finish which comprises preparing a surface presenting both porous and non-porous areas, and applying a nitrocellulose lacquer top-coat thereon containing a metallic powder and a dye, whereby the top-coat dries to the dyed metallic color over the non-porous areas, and to the undyed metallic color over the porous areas.

9. The method of producing a two-tone metallic effect which comprises partially sealing a porous base coat to form a surface presenting both porous and non-porous areas, and applying a top-coat thereon containing a metallic powder and a dye, whereby the top-coat dries to the dyed metallic color over the non-porous areas, and to the undyed metallic color over the porous areas.

10. The method of producing a two-tone metallic effect which comprises partially covering a non-porous first coat with a porous second coat, and applying a top-coat thereon containing a metallic powder and a dye, whereby the top-coat dries to the dyed metallic color over the non-porous areas, and to the undyed metallic color over the porous areas.

11. The method of producing a two-tone metallic effect which comprises covering a non-porous first coat with a crackled porous second coat, and applying a top-coat thereon containing a metallic powder and a dye, whereby the top-coat dries to the dyed metallic color over the non-porous areas, and to the undyed metallic color over the porous areas.

12. The method of producing a two-tone metallic effect which comprises spraying a crackle lacquer over a non-porous surface, allowing it to dry, and applying a top-coat thereon containing a metallic powder and a dye, whereby the top-coat dries to the dyed metallic color over the non-porous areas, and to the undyed metallic color over the crackle lacquer.

THEODORE A. NEUHAUS.